

## UNITED STATES PATENT OFFICE

2,294,287

COBALT RESINATE AND METHOD OF  
PRODUCING

Herschel A. Elliott, Wilmington, Del., assignor to  
Hercules Powder Company, Wilmington, Del.,  
a corporation of Delaware

No Drawing. Application September 4, 1941,  
Serial No. 409,537

11 Claims. (Cl. 260—100)

This invention relates to the production of fused cobalt resinates and more particularly to fused cobalt resinates of improved characteristics and to the method of production thereof.

Cobalt salts of wood or gum rosin have found wide usage as driers in paints and varnishes. Such salts have been made either by a precipitation method involving double decomposition of an alkali metal salt of rosin with a suitable cobalt compound, or by a fusion process involving fusion of the rosin with a reactive cobalt compound. By the precipitation method it has been possible to produce cobalt resinates containing up to the theoretical cobalt content for the neutral salt. By the fusion method, however, it has been impossible to introduce more than about 3% of cobalt due to the fact that blocking of the resinate occurs when about that amount of cobalt has become combined. For this reason the cobalt resinates produced commercially are usually prepared by the precipitation method. While such a method is more costly than the fusion method it has provided the only means of obtaining the desired higher cobalt contents.

It is an object of this invention to provide fused cobalt resinates of higher cobalt content than has been heretofore possible.

It is another object to provide fused cobalt resinates of high cobalt content which possess many improved characteristics.

It is a further object to provide a method of producing fused cobalt resinates of higher cobalt content than has been heretofore possible.

Other objects of the invention will appear hereinafter.

The above objects may be accomplished in accordance with this invention by fusing a hydrogenated rosin with a sufficient amount of a cobalt compound capable of reaction with the hydrogenated rosin, at a temperature in the range of about 200° C. to about 350° C. to give a cobalt resinate of the hydrogenated rosin having a cobalt content greater than the equivalent combining proportion of the hydrogenated rosin based on its acidity and as high as about 18% by weight. The theoretical cobalt content of a diresinate prepared from a rosin of theoretical acid number is 8.93%. This amount of cobalt thus represents the maximum obtainable in a resinate by the precipitation method and far exceeds the amount heretofore capable of introduction by a fusion procedure.

It has been found, in accordance with this invention, that by carrying out the fusion with hydrogenated rosin in place of ordinary rosin

and according to the described procedure, that clear homogeneous resinates may be prepared without the blocking disadvantage encountered in the production of cobalt resinates from ordinary rosins. Thus, by the process of this invention cobalt resinates containing more than the theoretical combining proportion of cobalt based on the acidity of the rosin and up to about twice the theoretical cobalt content of cobalt diresinate are made available.

In carrying out the fusion process of the invention a hydrogenated rosin is reacted with a cobalt compound capable of reaction therewith to provide a salt. Such a compound may be a basic cobalt compound or it may be a cobalt salt of a volatile weak acid or any other cobalt compound which under the fusion conditions liberates its cobalt. Suitable cobalt compounds are, for example, cobalt acetate, cobalt formate, cobalt lactate, cobalt butyrate, cobalt oxide, mixtures of cobalt oxide with a fatty acid as acetic acid, mixtures of cobalt oxide with a fatty acid cobalt salt as the acetate, etc. In using cobalt oxide it is usually desirable to employ it in admixture with a fatty acid or a fatty acid salt since the reactivity of the oxide alone is not sufficient to provide homogeneous resinates in the higher ranges of cobalt content described in accordance with this invention. As a catalytic material a small amount, such as 0.5 to 2% of the rosin, of calcium acetate or other fatty acid salt of calcium or a fatty acid salt of zinc, lead, manganese, etc., may be employed, if desired in conjunction with the cobalt compound.

The reaction is carried out by heating the hydrogenated rosin to a temperature in the range of about 200° C. to about 340° C. and adding the cobalt compound alone or in admixture with a catalytic metal compound such as a calcium salt either gradually or at one time, preferably while agitating the mixture. When the catalytic metal compound is used, satisfactory fusion takes place at temperatures as low as 200° C. but when the catalytic material is not employed it is usually desirable to employ a fusion temperature of at least about 275° C. At lower temperatures without the catalytic material there is a slight tendency to blocking in passing through the reaction stage representing formation of a resinate containing about 3 to 10% of combined cobalt. Considerable foaming accompanies the reaction and it is therefore preferable to agitate during the addition and to carry out the addition over an extended period. The foaming is more severe at the lower temperatures and reaction

is also slower. At temperatures above about 330° C. the reaction is very vigorous but the yield becomes diminished due to volatilization of light ends from the hydrogenated rosin. Temperatures of about 275 to about 330° C. are therefore preferable for the reaction.

The time of reaction required to combine the reactive cobalt compound with the hydrogenated rosin to produce the high metal content fused cobalt resinate is dependent on the temperature employed, the particular cobalt compound used, the degree of agitation, the particular amount of metal being introduced, as well as on other factors. Thus, the reaction time may be varied from about 10 minutes to several hours. It will be desirable to conduct the reaction in an inert atmosphere such as may be provided by carbon dioxide, nitrogen, etc., to prevent oxidation and discoloration of the hydrogenated rosin or the resinate at the elevated temperatures employed.

The hydrogenated rosin which may be employed in the process of the invention may be produced, as is well known in the art, by contacting wood or gum rosin or the acids contained therein with hydrogen and a suitable hydrogenation catalyst. Thus, by contacting rosin in a fluid condition with hydrogen in the presence of an activated base metal hydrogenation catalyst under a pressure in the range of about 200 to 15,000 pounds per square inch and at a temperature of about 125° C. to about 225° C. a hydrogenated product useful in this invention will be obtained. Hydrogenated rosin may also be obtained by contacting rosin dissolved in a suitable solvent with hydrogen and a noble metal hydrogenation catalyst, as for example platinum, palladium, etc., as is well known in the art. The hydrogenated rosin obtained by any of the above methods will have varying degrees of saturation depending on the actual conditions employed. For use in the present invention a hydrogenated rosin having a saturation value corresponding to at least about 50 per cent saturation of both double bonds of the rosin acid contained in the rosin will be preferred, although rosins of lower saturation may also be employed. Hydrogenated rosins having a saturation of about 50 to about 95 per cent of both double bonds will be particularly desirable in the production of the novel resinate of the invention. After hydrogenation the hydrogenated rosin may be subjected to vacuum distillation to remove the light end or to separate any particular fraction. If desired, it may be subjected to a refining treatment with a selective color-body solvent or absorbent as furfural, phenol, fuller's earth, etc. The hydrogenated rosin used will generally have an acid number above about 100 and preferably from about 135 to about 185.

The fused cobalt salts of hydrogenated rosin described in accordance with this invention will be considerably more useful in the commercial fields such as for example, as driers in paints or varnishes, in plastics, adhesives, printing inks, etc., due to the improved characteristics over prior cobalt resinate. Thus, they will contain a higher cobalt content than has been possible heretofore, which is a very desired advantage. They will also be less subject to oxidation and discoloration at both normal and elevated temperatures and will also be less subject to spontaneous ignition than the cobalt resinate prepared from ordinary rosin. They will be clear homogeneous resins and will be substantially free of precipitated or suspended matter.

The following specific examples are illustrative of the various embodiments of the invention:

*Example I*

5 One hundred parts by weight of a hydrogenated wood rosin saturated to the extent of 63% of both double bonds of the rosin acid contained therein and having an acid number of 158 and a drop melting point of 75° C. were melted and heated to a temperature of 240° C. in a nitrogen atmosphere. A mixture of 86 parts by weight of cobalt acetate and 9 parts by weight of calcium acetate was then added in small portions at a time with constant agitation and permitting the foaming to 10 subside before each subsequent addition. The reaction temperature was raised during the addition to a maximum of 330° C. A total addition time of 95 minutes was required. The cobalt resinate obtained was a clear homogeneous resin having a drop melting point of 220° C. and a cobalt content of 17% and a calcium content of 2%.

*Example II*

25 One hundred and ten parts by weight of hydrogenated gum rosin having a saturation of 60% of both double bonds of the rosin acid contained therein, an acid number of 155 and a drop melting point of 79° C. were melted and heated to a temperature of 255° C. in a nitrogen atmosphere. A mixture of 71 parts by weight of cobalt acetate and 10 parts by weight of calcium acetate was then added gradually in small portions at a time with constant agitation and while permitting the reaction to subside before each subsequent addition. The reaction temperature was raised gradually during the addition to a maximum of 325° C. The fused cobalt resinate obtained had a melting point of 215° C., a cobalt content of 13.3% and a calcium content of 2%. It was a clear homogeneous resin.

*Example III*

30 Using the hydrogenated wood rosin described in Example I, 400 parts by weight of the rosin were melted and heated to a temperature of 280° C. in a carbon dioxide atmosphere. A mixture of 167 parts by weight of cobalt acetate and 36 parts by weight of calcium acetate was then added gradually in small portions at a time with agitation. The reaction temperature was raised gradually to a maximum of 310° C. during the addition. A total addition time of 70 minutes was employed. The cobalt resinate obtained had a drop melting point of 200° C., a cobalt content of 9%, and a calcium content of 2%.

35 It will be understood that the details and examples hereinbefore set forth are illustrative only and that the invention as broadly described and claimed is in no way limited thereby.

40 What I claim and desire to protect by Letters Patent is:

1. A cobalt resinate of a hydrogenated rosin having a cobalt content greater than the equivalent combining proportion of the hydrogenated rosin but not in excess of about 18% by weight.

2. A cobalt resinate of a hydrogenated rosin saturated to the extent of at least 50% of both double bonds of the rosin acid contained therein and having a cobalt content greater than the equivalent combining proportion of the hydrogenated rosin but not in excess of about 18% by weight.

3. A cobalt resinate of a hydrogenated wood rosin having a cobalt content greater than the equivalent combining proportion of the hydro-

genated rosin but not in excess of about 18% by weight.

4. A cobalt resinate of a hydrogenated gum rosin having a cobalt content greater than the equivalent combining proportion of the hydrogenated rosin but not in excess of about 18% by weight.

5. The method of producing a cobalt resinate of a hydrogenated rosin having a cobalt content greater than the equivalent combining proportion of the hydrogenated rosin but not in excess of about 18% by weight, which comprises fusing a hydrogenated rosin with a cobalt compound capable of reaction with the hydrogenated rosin, in an amount sufficient to give a resinate of the above defined cobalt content at a temperature within the range of about 200° C. to about 350° C.

6. The method of producing a cobalt resinate of a hydrogenated rosin having a cobalt content greater than the equivalent combining proportion of the hydrogenated rosin but not in excess of about 18% by weight, which comprises fusing a hydrogenated rosin with a cobalt compound capable of reaction with the hydrogenated rosin, in an amount sufficient to give a resinate of the above defined cobalt content and in the presence of a catalytic metal compound at a temperature within the range of about 200° C. to about 350° C.

7. The method of producing a cobalt resinate of a hydrogenated rosin having a cobalt content greater than the equivalent combining proportion of the hydrogenated rosin but not in excess of about 18% by weight, which comprises fusing a hydrogenated rosin with a cobalt compound capable of reaction with the hydrogenated rosin, in an amount sufficient to give a resinate of the above defined cobalt content and in the presence of a small amount of a calcium salt as catalyst at a temperature within the range of about 200° C. to about 350° C.

8. The method of producing a cobalt resinate of a hydrogenated rosin having a cobalt content greater than the equivalent combining propor-

tion of the hydrogenated rosin but not in excess of about 18% by weight, which comprises fusing a hydrogenated rosin with a cobalt compound capable of reaction with the hydrogenated rosin, in an amount sufficient to give a resinate of the above defined cobalt content at a temperature within the range of about 275° C. to about 330° C.

9. The method of producing a cobalt resinate of a hydrogenated rosin having a cobalt content greater than the equivalent combining proportion of the hydrogenated rosin but not in excess of about 18% by weight, which comprises fusing a hydrogenated rosin with cobalt acetate in an amount sufficient to give a resinate of the above defined cobalt content and in the presence of a small amount of calcium acetate as catalyst at a temperature within the range of about 275° C. to about 330° C.

10. The method of producing a cobalt resinate of a hydrogenated rosin having a cobalt content greater than the equivalent combining proportion of the hydrogenated rosin but not in excess of about 18% by weight, which comprises fusing a hydrogenated rosin with a mixture of cobalt oxide and cobalt acetate in an amount sufficient to give a resinate of the above defined cobalt content and in the presence of a small amount of calcium acetate as catalyst at a temperature within the range of about 275° C. to about 330° C.

11. The method of producing a cobalt resinate of a hydrogenated rosin having a cobalt content greater than the equivalent combining proportion of the hydrogenated rosin but not in excess of about 18% by weight, which comprises fusing a hydrogenated rosin with a mixture of cobalt oxide and acetic acid in an amount sufficient to give a resinate of the above defined cobalt content and in the presence of a small amount of calcium acetate as catalyst at a temperature within the range of about 275° C. to about 330° C.

HERSCHEL A. ELLIOTT.